

June 7, 1966

L. D. CAUL ET AL

3,254,357

COMBINED SCRUBBING AND POLISHING PAD

Filed Aug. 10, 1961



Fig. 1



Fig. 2



Fig. 3

INVENTORS  
LAWRENCE D. CAUL  
JOSEPH R. O'NEIL JR.  
BY

*H.W. Boundell*

ATTORNEY

1

3,254,357

**COMBINED SCRUBBING AND POLISHING PAD**  
 Lawrence D. Caul, Buffalo, and Joseph R. O'Neil, Jr.,  
 Youngstown, N.Y., assignors to The Carborundum  
 Company, Niagara Falls, N.Y., a corporation of Delaware

Filed Aug. 10, 1961, Ser. No. 130,587  
 9 Claims. (Cl. 15—118)

This invention relates to surface maintenance pads, and more particularly to a new and improved pad for both scrubbing and polishing surfaces such as waxed floors.

While many types of pads have been employed for maintaining floor surfaces, they have certain inherent characteristics which limit their effectiveness and efficiency in the scrubbing and polishing of floors. The most common material used for such pads has been steel wool, which has the undesirable characteristics of staining, rapid wear, poor strength, and rapid deterioration by oxidation as rust forms, particularly in the presence of water and wetting agents. In addition, steel wool has a tendency to throw the cleaning solution away from the rotary scrubbing machine, which substantially reduces the efficiency of the operation, and causes splattering and soiling of walls and baseboards.

Numerous attempts have been made to overcome these objectionable characteristics of steel wool pads by utilizing synthetic plastic fibers of either thermoplastic or thermosetting type. However, in themselves, the thermoset fibers are too stiff and brittle for effective polishing action, while the thermoplastic fibers are too soft for scrubbing and tend to become depressed and take a permanent set when so used. Further, in order to provide the desired abrading action, it has been thought to be necessary to coat and/or impregnate such fibers with abrasive particles, which adds considerably to the cost of manufacturing such pads. Moreover, it has been found that the addition of such abrasive particles has not produced any marked increase in the efficiency and effectiveness of the polishing or scrubbing operations. In addition, such prior art pads have usually been provided with only a single working surface or side, which further limits their usefulness to either one or the other type of operation, and up to the present, no pad has been commercially produced which is equally effective for both scrubbing and polishing purposes.

Accordingly, it is a primary object of the present invention to provide a new and improved pad which is so constructed and designed as to have a scrubbing side and a polishing side for maximum efficiency and effectiveness in each type of operation.

Another primary object is to provide such a pad which is so constructed and designed as to completely eliminate the need for abrasive particles of any kind, yet is most effective and efficient for its intended purposes, while being more economical to manufacture than pads containing such abrasive particles.

Another object is to provide such a pad which utilizes the greater inherent resiliency and toughness of curled animal hair over synthetic plastic fibers, as well as the ability of such hair to recover its natural loft following removal of moisture by drying, as opposed to moisture impervious synthetic fibers such as nylon, which lack such memory.

Other objects and advantages of the invention will become apparent upon consideration of the following detailed description and accompanying drawing wherein:

FIG. 1 is a perspective view of a combined scrubbing and polishing pad constituting a preferred embodiment of the invention, and arranged with its scrubbing side uppermost;

FIG. 2 is a greatly enlarged, fragmentary horizontal

2

sectional view of the scrubbing side of the pad of FIG. 1, and illustrating the interrelationship of the curled animal hairs, the elastomeric binder and the thermoset resinous binder, and

5 FIG. 3 is an enlarged fragmentary vertical sectional view taken on line 3—3 of FIG. 1, and illustrating by deeper shading the scrubbing side and by lighter shading the polishing side of the pad.

Referring to the drawing, and particularly FIGS. 1 and 2, a preferred embodiment of the inventive pad is generally indicated at 10. Such pad is preferably of circular configuration and is suitably die cut from a sheet of curled animal hair felt of open structure, i.e., with voids 11 between and among the individual hairs 12. Preferably, 15 throughout the thickness of the felt pad, the individual hairs 12 are coated by a cured elastomer 13, which forms resilient globules 14 bonding the individual hairs at their intersections. In addition, the individual hairs 12 are further coated with one or more coats of a thermoset or 20 heat-hardened resin 15 which covers the elastomer and forms hard nodules 16 over globules 14. As will be apparent, such nodules 16 further bond the individual hairs 12 at their intersections. However, the resin is permitted to impregnate the felt pad 10 throughout only a portion of 25 its thickness as best illustrated in FIGS. 1 and 3 by the deeper shaded areas. As a consequence, the pad 10 is provided with a stiff scrubbing side 17 which presents a scrubbing surface 18 characterized by hairs 12 which have been coated with a relatively hard outer resin forming 30 hard nodules 16 at the intersections of such hairs. It has been found that the combination of the inherently tough and resilient animal hairs 12 and the hard resin coating 13 and nodules 16 provides a most effective and efficient 35 scrubbing surface 18, with the nodules 16 providing sufficient aggressive action, thereby completely eliminating the need for abrasive particles formerly thought to be required.

At the same time, the inventive pad 10 is also provided with a flexible polishing side 19 indicated by lighter shading in FIGS. 1 and 3 and which presents a polishing surface 20 which is relatively soft and resilient. Once again, it has been found that the globules 14 (which would be exposed in the polishing side) provide sufficient aggressive action, whereas no abrasive particles are required for 45 effective polishing action either. In addition, it has been found that the underlying elastomeric coating 13 and globules 14 provide a resilient base for the hard and relatively brittle resin coating 15 and nodules 16, and this resilient base reduces somewhat the tendency of the harder, more brittle resin to wear unduly rapidly during 50 the scrubbing operation. Moreover, by employing the curled animal hair fibers 12, as the resinous and elastomeric coatings wear away, and such hairs absorb moisture, they nevertheless have the inherent ability to recover 55 their original toughness and resiliency after the moisture has been removed by drying. This characteristic of the animal hair has a definite advantage over moisture impervious synthetic fibers such as nylon, which do not have such memory.

60 A typical application of the inventive pad involves placing the pad on a floor to be cleaned with the scrubbing surface 18 down in contact with the floor, and a scrubbing machine (not shown) provided with a Tampico fiber brush or the like (not shown) is then placed upon the pad 10. With water and/or other suitable cleaning agent applied to the floor, the machine is started, and its weight causes the pad to rotate in contact with the floor to effect the desired scrubbing action. When this scrubbing operation is complete, a conventional wax or polish is applied to the floor, and the inventive pad, which has 65 been rinsed to remove dirt or scrubbing material and then partly dried, is replaced under the machine as 70 de-

scribed above, but with the polishing surface 20 contacting the floor to provide the desired polishing action.

A wide variety of animal hair is applicable for use in the inventive pad, but cattle, hog and horse hair including mane hair are preferred. Such hair is employed in a curled state, and the particular species listed are preferred because they provide the desired open felt structure, and possess the inherent toughness, resiliency and ability to recover such characteristics following drying. Likewise, various thermosetting or heat-hardening synthetic resins may be used as the bonding material for the scrubbing side of the inventive pad. Typical of such resins are phenolics, phenolics with acetals, urea formaldehyde, acrylates, epoxies, epoxy-polyamides and the like. In addition, various elastomers such as natural rubber, 10 butadiene styrene polymers, butadiene acrylonitrile polymers, polyvinyl chloride and the like may be used as the binding material for the polishing side of the inventive pad.

Inasmuch as it is not necessary to employ abrasive 20 particles in the inventive pad, there is no danger of scratching or marring the surface being worked on, especially when being cleaned during the scrubbing operation. In addition, the polishing side 19 has been found to be especially suitable for the buffing of harder waxes. By 25 way of comparison, nylon which has been used for this purpose in the past, has been found to be satisfactory on the softer waxes, but does not give sufficient buffing action on the harder waxes.

In manufacturing the inventive pad, it is preferred that the hair pad be sprayed or roll-coated so that it is impregnated with the elastomeric bonding material throughout its thickness. However, this is not absolutely necessary, as the thermosetting resin can be relied upon to bind the individual hairs together at their intersections throughout the scrubbing side of the pad. Even so, complete impregnation by the elastomeric binding material is preferred because it provides a resilient base for the harder and more brittle resin in the scrubbing side of the pad, for a softer scrubbing action and increased wear of the 40 scrubbing surfaces.

For most floor maintenance applications, the inventive pad will vary in thickness from about  $\frac{3}{16}$ " to about 1", and in weight from about 1 ounce per square foot to approximately 5 ounces per square foot, these values being given for a so called "raw" pad which has been impregnated throughout its thickness with the elastomer prior to application of the resin. Further, it has been found that a pad of about  $\frac{3}{4}$ " nominal thickness and weighing about 3 ounces per square foot is a most effective scrubbing and 45 polishing product.

The following example will highlight the present invention, and illustrate in detail a preferred embodiment thereof.

#### Example

A  $\frac{3}{4}$ " thick, random-oriented air-laid pad comprising 20% by weight of curled cattle hair and 80% by weight of curled hog hair was treated with an epoxy-polyamide resin to provide a maintenance pad in accordance with the present invention. The "raw" impregnated pad had a weight of 3 ounces per square foot and the curled hairs thereof were coated and bonded together at their points of intersection by cured neoprene latex.

The "raw" pad was placed on a horizontal support and sprayed to a penetration depth of  $\frac{3}{16}$ " with the following composition:

|                                                                                                                                                                                                                      | Parts by weight |
|----------------------------------------------------------------------------------------------------------------------------------------------------------------------------------------------------------------------|-----------------|
| Diglycidyl ether of p,p'-isopropylidenediphenol                                                                                                                                                                      | 100             |
| Polyamide reaction product of an aliphatic amine and a monocarboxylic acid; having an equivalent weight of 90 and a viscosity at 77° F. of 150-400 centipoises (Epi-Cure 855, a product of the Jones-Dabney Company) | 70              |
|                                                                                                                                                                                                                      | 50 75           |

The resin composition was sprayed on the top side of the pad at a rate of about 0.33 pound per square yard. Thereafter, an additional coat of adhesive was applied at a rate of about 0.20 pound per square yard. After the second coating operation was completed, the pad was heated in an oven to a temperature of 250° F. for a period of about 8 minutes to cure the resin. Thereafter the pad was flexed to render it more flexible.

Penetration of the resin into the pad was controlled to leave a  $\frac{1}{16}$ " portion uncoated at the base of the pad, which allowed this side of the pad to be used for the buffing of waxes as well as to provide a cushion to allow the pad to adjust to and effectively treat uneven floor surfaces during either scrubbing or polishing thereof.

The product displayed a most effective and efficient, yet "velvet" or "soft" scrubbing action when employed to strip old wax and soil from an asphalt tile floor surface in conjunction with an electric rotary floor treating machine employing a commercial floor cleaning detergent in water as the cleaning agent. Likewise, when turned over, the product was most effective and efficient in buffing to a high lustre a hard commercial wax applied to said floor by the aforesaid machine following rinsing and drying of the product.

It will now be seen how the invention accomplishes its various objectives, and the numerous advantages possessed by the inventive pad will also be apparent. While the invention has been described and illustrated herein with respect to certain preferred embodiments, it is to be understood that various changes and modifications may be made in the invention by those skilled in the art without departing from the inventive concept, the scope of which is to be determined by the appended claims.

We claim:

1. A cleaning pad which consists of an open, porous felt of randomly arranged, curled animal hair, the individual hair fibers of said felt being bonded throughout said pad at their points of intersection by a cured elastomer, said pad having a stiff, scrubbing side in which the individual hair fibers are coated with a thermoset resin which also covers said elastomer and provides a further bond for said fibers at their points of intersection, said thermoset resin extending through only a portion of the thickness of said felt, and a flexible side free from said resin formed by the remaining portion of the thickness of said felt, said pad being free from abrasive throughout its thickness.

2. A cleaning pad as set forth in claim 1 in which said curled hair consists of a mixture of curled cattle hair and curled hog hair.

3. A cleaning pad as set forth in claim 1 in which said elastomer forms resilient globules at the intersections of the curled hair fibers and said thermoset resin forms hard nodules over said globules only in the stiff, scrubbing, side of said pad.

4. A cleaning pad as set forth in claim 3 in which said curled hair consists of a mixture of curled cattle hair and curled hog hair.

5. A cleaning pad as set forth in claim 1 in which said elastomer forms a coating over substantially all of the curled hair fibers as well as bonding them at their points of intersection and said thermoset resin further coats the curled hair throughout the thickness of said scrubbing side.

6. A cleaning pad as set forth in claim 5 in which said curled hair consists of a mixture of curled cattle hair and curled hog hair.

7. A cleaning pad as set forth in claim 5 in which said cured elastomer forms resilient globules at the intersections of said curled hair fibers and in which, in the scrubbing side of said pad, said thermoset resin forms hard modules over said globules.

8. A cleaning pad as set forth in claim 7 in which said curled hair consists of a mixture of curled cattle hair and curled hog hair.

9. A cleaning pad which consists of an open, porous felt of randomly arranged, curled animal hair, the individual hair fibers of said felt being bonded throughout said pad at their points of intersection by a cured elastomer, said pad having a stiff, scrubbing side in which the individual hair fibers are coated with an epoxy resin which also covers said elastomer and provides a further bond for said fibers at their points of intersection, said epoxy resin extending through only a portion of the thickness of said felt, and a flexible side free from said resin formed by the remaining portion of the thickness of said felt, said pad being free from abrasive throughout its thickness.

10

## References Cited by the Examiner

## UNITED STATES PATENTS

|           |        |        |       |        |
|-----------|--------|--------|-------|--------|
| 1,454,049 | 5/1923 | Genung | ----- | 28-79  |
| 2,113,452 | 4/1938 | Long   | ----- | 15-105 |

|             |         |                              |
|-------------|---------|------------------------------|
| 2,232,945   | 2/1941  | Hately.                      |
| 2,526,468   | 10/1950 | Frye ----- 15-210            |
| 2,803,577   | 8/1957  | Colt et al. ----- 156-588 X  |
| 2,958,593   | 11/1960 | Hoover et al. ----- 15-209.5 |
| 5 2,972,554 | 2/1961  | Muskat et al. ----- 154-54 X |
| 3,171,151   | 3/1965  | Sickle et al. ----- 15-209.5 |

## FOREIGN PATENTS

181,389 3/1955 Austria.

## OTHER REFERENCES

Article in "Plastics Technology," July 1957, vol. III, No. 7, page 579.

15 DANIEL BLUM, Primary Examiner.

S. JAMES, CHARLES A. WILLMUTH, Examiners.